

# UNITED STATES PATENT OFFICE.

SIDNEY D. WELLS, OF MADISON, WISCONSIN, DEDICATED, BY MESNE ASSIGNMENTS, TO THE GOVERNMENT OF THE UNITED STATES AND TO THE PEOPLE OF THE UNITED STATES.

## MANUFACTURE OF PAPER-PULP.

1,269,350.

Specification of Letters Patent. Patented June 11, 1918.

No Drawing.

Application filed April 30, 1918. Serial No. 231,735.

(DEDICATED TO THE PUBLIC.)

*To all whom it may concern:*

Be it known that I, SIDNEY D. WELLS, a citizen of the United State, residing at Madison, in the county of Dane and State 5 of Wisconsin, (whose post-office address is R. F. D. No. 4, Madison, Wisconsin,) have invented a new and useful Improvement in the Manufacture of Paper-Pulp.

This application is made under the act of 10 March 3, 1883, chapter 143 (22 Stat. 625), and the invention herein described and claimed may be used by the Government of the United States, or any of its officers or employees, in the prosecution of work for 15 the Government, or any person in the United States, without payment to me of any royalty thereon.

My invention relates to the manufacture of paper pulp by alkaline processes from 20 wood and other materials of a fibrous nature whereby the yield and quality of pulp obtained is increased while the consumption of chemical and duration of cooking is decreased.

25 The object of the invention is to add water to the charge during the cooking and thereby diminish the action of the cooking liquors on the cellulose while the action of the cooking liquors on the incrusting matter remains the same.

In the practice of the invention, the process is carried out in the following manner: The material of a fibrous nature is prepared by any of the means now practised in the art 35 and charged into the digester as in common practice. The cooking liquor is also added and any preliminary operations such as steaming, distillation of volatile oils, preliminary penetration, and the like, may be 40 followed as desired. Steam is then admitted to the digester and the contents are brought up to the desired cooking pressure. When the temperature in the digester is sufficient to cause the cooking liquor actively

45 to attack the incrusting material, water is admitted into the digester, in addition to the moisture carried in by the steam, in sufficient quantity, whereby the action of the cooking liquors on the cellulose is diminished while the action of the cooking liquors 50 on the incrusting matter remains the same.

The addition of water in this manner operates to increase not only the yield but also the quality of the pulp produced. The cook is carried out by any of the means commonly practised in the art. I have found that in cooking poplar by the soda process, the yield of pulp obtained was increased 9 per cent. by adding moisture with the steam so that the total moisture added amounted 60 to 1500 gallons of water per cord of wood. Any increase over this does not materially increase the yield.

The increase in yield found obtainable with the introduction of moisture is not obtainable by adding moisture at the beginning of the cook by means of using more dilute cooking liquors.

The addition of the moisture may be secured either by admitting water with the 70 steam, by the use of wet steam, or by adding water into the digester through a separate inlet.

Having thus described my invention, I claim:

1. A process of cooking wood or other fibrous material for the production of paper pulp in which the desired amount of moisture is introduced to the digester during the cook in direct combination with the steam 80 whereby the cellulose is protected to a marked degree from the action of the cooking liquors while their action on the incrusting matter is in no way diminished.

2. A process of cooking wood or other fibrous material for the production of paper pulp in which the desired amount of moisture is introduced into the digester during the cooking by using wet steam carrying the desired amount of moisture in excess of that 90 in saturated steam, whereby the cellulose is protected to a marked degree from the action of the cooking liquors while their action on the incrusting matter is in no way diminished.

3. A process of cooking wood or other fibrous material for the production of paper pulp in which the desired amount of moisture over that admitted in the steam is introduced into the digester during the cook 100 by a separate inlet whereby the cellulose is protected to a marked degree from the ac-

tion of the cooking liquors while their action on the incrusting matter is in no way diminished.

4. A process of cooking wood or other fibrous material for the production of paper pulp in which the desired amount of moisture is introduced into the digester during the cook by any means whatever, whereby the cellulose is protected to a marked degree

from the action of the cooking liquors while 10 their action on the incrusting matter is in no way diminished.

In testimony, I affix my signature in the presence of two subscribing witnesses.

SIDNEY D. WELLS.

Witnesses:

OTTO KRESS,  
G. C. McNAUGHTON.